

3,634,262

## PROCESS AND COMPOSITIONS FOR TREATING ALUMINUM AND ALUMINUM ALLOYS

John J. Grunwald, New Haven, and Edmund E. Horner,  
Watertown, Conn., assignors to MacDermid, Incorporated,  
Waterbury, Conn.

No Drawing. Filed May 13, 1970. Ser. No. 37,013  
Int. Cl. C11d 7/54

U.S. CL. 252—100

15 Claims

### ABSTRACT OF THE DISCLOSURE

Aluminum and aluminum alloy surfaces are prepared for metal finishing operations such as anodizing, painting, bright dipping etc., by immersing them for about 1 to about 10 minutes at a temperature of about 60° to about 170° F. in an acidic solution of a peroxydiphosphate compound, such as potassium peroxydiphosphate. Optionally, the solution may also contain a fluoride salt.

This invention relates to the surface preparation of aluminum and aluminum alloys for subsequent metal finishing operations such as painting, anodizing, plating, bright dipping, welding, chromating, etc. More particularly, this invention relates to novel acidic compositions containing ammonium peroxydiphosphate or peroxydiphosphates of the alkali metals and the alkaline earth metals and to a process for deoxidizing and desmutting aluminum surfaces subsequent to the final metal finishing operation.

It is an important procedure in the aluminum finishing industry, prior to the finishing operations mentioned above, to remove the ever-present oxide film which forms on the surface of aluminum alloys on atmospheric exposure. A typical method employed in the past by which this is achieved is to immerse the previously degreased aluminum object in a suitable deoxidizing solution, which usually contains oxidizing agents such as chromic acid, chromates or dichromates, nitric acid or a mixture of these materials in well defined proportions. Their function is to replace this tenacious oxide film on the aluminum alloy by another film more suitable for subsequent treatments.

The use of chromic acid or any other chrome base deoxidizing solution in the finishing industry creates waste disposal difficulties since these formulations must be treated chemically before they can be disposed of safely. Also the use of chromic acid in certain finishing shops may cause contamination of rinsing waters, bright dips, anodizing and plating solutions. Furthermore, the use of nitric acid is always accompanied by obnoxious fumes which makes for uncomfortable and health hazardous conditions as well as corrosive action in many plating installations.

Another procedure frequently used heretofore in the aluminum finishing industry as a preparatory step, prior to the finishing treatments, consists of etching the aluminum alloy in a suitable alkaline solution, thereby removing substantial amounts of surface metal. During this etching process, certain alloying elements of the aluminum, which are insoluble in the etching solution, will cover the surface in the form of a loose coating forming an unsatisfactory basis for further treatment, and care must therefore be taken to see that this loose coating is completely removed. This phenomenon is known in the industry as smut formation, and removal of the smut is also covered by the term "deoxidizing" as it is used in practice and in the present specification and appended claims.

It is therefore a primary object of this invention to provide a novel deoxidizing solution which is free of waste treatment difficulties and wherein the ingredients are readily controllable at the room operating temperature of the solution; also to provide a solution compatible with bright dip and anodizing solutions. It is a further object of the invention to eliminate adherent films on the articles undergoing treatment and the production of offensive fumes and insoluble residues in the bath, which

5 disadvantages have inherently characterized prior aluminum deoxidizing and desmutting operations. Among other advantages of the treatment herein disclosed is the fact that the bath components used are physiologically safe, which makes them well suited for treating aluminum objects to be used in the food industry. It is found that the deoxidizing action of the novel bath composition here disclosed is considerably faster than other existing proprietary deoxidizers. Other features and advantages of the invention will be discussed as the description proceeds.

10 As previously pointed out, the novel deoxidizing and desmutting compositions of this invention contain at least one peroxydiphosphate compound which by itself in aqueous solution regardless of the concentration will not perform as a deoxidizer or deoxidizer-desmutter of aluminum or aluminum alloys. Surprisingly, the novel deoxidizing and desmutting solutions of this invention which comprise aqueous solutions of a peroxydiphosphate compound selected from the group consisting of ammonium peroxydiphosphate, an alkali metal peroxydiphosphate 15 and an alkaline earth metal, and certain acids or acid salts thereof in sufficient amount to provide a solution pH of not over 3.0, are excellent deoxidizing and desmutting compositions. The concentration of the peroxydiphosphate compound which can be varied over a wide range generally will be from about 18 grams per liter up to saturation. Such solutions provide excellent deoxidizing and desmutting action on aluminum and all aluminum alloys with the exception of those alloys having a high silicon content. These novel aqueous solutions 20 are especially useful in deoxidizing and desmutting wrought aluminum and wrought aluminum alloys. Further, it has been found that casting alloys with silicon content not in excess of 1%, can be handled with these same solutions provided a fluoride anion is included as 25 one of the ingredients.

In the deoxidizing-desmutting process of this invention, the peroxydiphosphates react with the aluminum or its alloying elements and are reduced to the orthophosphates. Thus, the bath after being exhausted, can be conveniently disposed of after neutralization as in the case of any other spent acid solution.

Furthermore, introduction of a suitable wetting agent such as any of the well-known surface tension depressing 30 ionic or nonionic materials, is found to be of great assistance in removing oxide films from aluminum strip processed in continuous operation, wherein the aluminum strip is moved at high speed through a trough containing the deoxidizing solution and then through a rinsing trough. Large quantities of aluminum strip can be processed during short periods of time in such manner. Such treatments are impossible with chrome type deoxidizers which require very abundant rinsing that cannot be provided in a continuous operation.

Another advantage of this formulation is that it will 35 not dimensionally alter or affect aluminum objects that are immersed, even for very prolonged periods of time.

Alkali metal peroxydiphosphates which can be employed in formulating the novel solutions of this invention include sodium, potassium and lithium peroxydiphosphates while the useful alkaline earth metal peroxydiphosphates include calcium and magnesium.

As previously pointed out it is sometimes advantageous to add a fluoride anion to the novel solutions of this invention and this is especially true with regard to aluminum alloys which contain a considerable amount of silicon such as Type 6061, 6063, etc. A wide variety of soluble fluoride compounds can be employed although it is preferred to utilize a fluoride compound selected from the group consisting of  $\text{NaF}$ ,  $\text{NaHF}_2$ ,  $\text{NH}_4\text{HF}_2$ ,  $\text{Na}_2\text{SiF}_6$ ,  $\text{HF}$ ,  $\text{HBF}_4$ ,  $\text{KF}$ ,  $\text{KHF}_2$ ,  $\text{NaHF}_4$ ,  $\text{NH}_4\text{F}$ ,  $\text{K}_2\text{SiF}_6$ ,  $\text{FeF}_3$  and mixtures thereof. Generally, sufficient soluble fluoride compound is added to provide a fluoride ion concentration in the aqueous solution of from 0 to about 6 grams per liter.

Acids useful in preparing the novel compositions of his invention include sulfuric, phosphoric, sulfamic, and mixtures thereof; acid salts of these same acids, such as sodium bisulfate, potassium bisulfate and mixtures thereof. Preferably, the acid used in preparing the novel deoxidizing solutions is sulfuric acid. Sufficient acid, acid salt, or a mixture of these two materials is added to the novel bath composition to provide a pH of not more than 1.0.

A complete deoxidizing process for aluminum and aluminum alloys utilizing the novel acidic aqueous peroxydiphosphate solutions of this invention together with the usual cleaning and etching steps is as follows:

#### PROCESS I

- 1) 3 to 5-minute immersion in a non-etch aluminum soak cleaner at a concentration of 8 to 10 oz./gal. and at 160° to 180° F.,
- 2) 30-second cold water rinse,
- 3) 1 to 3-minute immersion in an alkaline etchant at a concentration of 8 to 10 oz./gal., temperature 160° to 180° F.,
- 4) 30-second cold water rinse,
- 5) 1 to 10-minute immersion in an acidic aqueous potassium peroxydiphosphate solution at a temperature about 60° to about 170° F. to desmut and deoxidize the aluminum,
- 6) 30-second cold water rinse, and
- 7) subsequent finishing operations such as: anodizing, chromating, etc.

A similar process in which the etching step is not employed comprises the following steps:

#### PROCESS II

- 1) 3 to 5-minutes immersion in an alkaline non-etch aluminum soak cleaner at a concentration of 8 to 10 oz./gal. and at a temperature of about 160° to 180° F.,
- 2) 30-second cold water rinse,
- 3) 1 to 5-minute immersion in an acidic aqueous potassium peroxydiphosphate solution at a temperature of about 60° to about 170° F., to deoxidize the aluminum,
- 4) 30-second cold water rinse, and
- 5) subsequent finishing operations such as: anodizing, chromating, etc.

Generally, the metal surface is immersed in the acidic aqueous peroxydiphosphate bath for about 1 to about 0 minutes or more and preferably for about 1 to about 5 minutes. A useful deoxidizer-desmutter solution not only must remove smut and deoxidize the aluminum but must also not have a detrimental effect on the metal surface with extended immersion times. These requirements are met in the novel acidic peroxydiphosphate solutions of this invention.

In another aspect, this invention relates to dry compositions which can be dissolved with mixing in water to form deoxidizing and desmutting solutions of the type previously described. The dry compositions of this invention comprise (1) a water soluble peroxydiphosphate salt selected from the group consisting of ammonium peroxydiphosphate, an alkali metal peroxydiphosphate and an alkaline earth metal peroxydiphosphate, (2) an acid salt of sulfuric acid and, optionally, a soluble fluoride

salt. Generally, the novel dry compositions of this invention will contain the following ingredients in approximate percentages indicated below:

| Ingredients:               | Percent by weight |
|----------------------------|-------------------|
| Peroxydiphosphate salt     | 5-20              |
| Acid salt of sulfuric acid | 77-95             |
| Fluoride salt              | 0-3               |

Any of the peroxydiphosphate salts, acid salts of sulfuric acid, and fluoride salts previously described in connection with the description of the novel deoxidizing and desmutting solutions of this invention can be employed in preparing the novel dry compositions.

The pH of the aqueous solution prepared from the dry compositions must be less than 3.0 if the resulting solution is to operate effectively as a deoxidizing and desmutting composition. However, if adjustment of the pH is required, it can be conveniently carried out through the addition of sulfuric acid in any needed amount.

Dry powder compositions offer a number of advantages over the liquid compositions especially with regard to easier handling and lower shipping weights. Further, the use of such dry compositions offers the additional advantage of elimination of the majority of the weighing out or measuring operations thus further reducing the possibility of faulty make-up.

The following examples illustrate various embodiments of this invention and are to be considered not limitative.

#### Example I

An aqueous solution containing the following ingredients in the amounts indicated, in addition to water, was prepared:

- 35 Potassium peroxydiphosphate ( $\text{K}_4\text{P}_2\text{O}_8$ )—120 g./l.
- Sulfuric acid (66° Bé.)—40 ml./l.
- pH—<3.0

Aluminum objects prepared from Type 7075 aluminum alloy (Analysis: 1.6% Cu, 2.5% Mg, 5.6% Zn, 0.2% Cr—balance Al plus impurities) were immersed in a non-etch aluminum soak cleaner having a concentration of 8 oz./gal. at 170° F., rinsed in cold water, immersed in an alkaline etchant at a concentration of 10 oz./gal. at 160° F. for 3 minutes during which time a heavy dark smut developed on the surface of the aluminum objects, again rinsed in cold water, immersed in the above-described solution of potassium peroxydiphosphate at a temperature of 70° F. for 3 minutes; and then rinsed for 30 seconds in cold water. The thus-treated aluminum objects exhibited light and smut-free surfaces which provide an excellent base for subsequent finishing operations such as painting, dyeing, chromating, etc.

#### Example II

In this example an aqueous solution having the following composition is employed in treating the surfaces of aluminum objects:

- 60 Lithium peroxydiphosphate ( $\text{Li}_4\text{P}_2\text{O}_8$ )—105 g./l.
- Sulfuric acid (66° Bé.)—60 ml./l.
- pH—<3.0

Utilizing the same procedure and cleaning and etching solutions utilized in Example I, aluminum objects of Type 2024 alloy (Analysis: 4.5% Cu, 0.6% Mn, 1.5% Mg—balance Al plus impurities) are desmuted and deoxidized in the above-described lithium peroxydiphosphate solution. The resulting aluminum alloy objects possess light surfaces completely free of smut which are highly satisfactory for further finishing.

#### Example III

In this example articles made of an aluminum alloy having a substantial silicon content are deoxidized and

desmutted using an aqueous solution of the following composition:

Ammonium peroxydiphosphate  $((\text{NH}_4)_4\text{P}_2\text{O}_8)$ —140 g./l.  
Phosphoric acid (85% strength)—30 ml./l.  
Sulfuric acid (66° Bé.)—60 ml./l.  
pH—<3.0

Aluminum articles manufactured from Type 6061 alloy (Analysis: 0.25% Cu, 0.6% Si, 1.0% Mg and 0.25% Cr—base Al plus impurities) are first cleaned by immersion for 5 minutes at 160° F. in an alkaline non-etch aluminum soak cleaner at a concentration of 8.5 oz./gal., rinsed in cold water for 30 seconds, immersed in the peroxydiphosphate solution previously prepared in this example for 25 minutes at 80° F. and rinsed again for about 30 seconds in cold water. The thus-treated articles exhibit aluminum surfaces which are of excellent appearance and well-suited for further finishing operations such as phosphating, bright dipping, etc.

#### Examples IV—XII

In these examples articles prepared from Type 6061 and 6063 aluminum alloys which contain substantial quantities of silicon were cleaned, etched and then treated at a temperature of 72° F. in an acidic aqueous peroxydiphosphate solution in the same manner as described in Example I. Pertinent data relating to the acidic peroxydiphosphate compositions utilized in these examples is shown in Table 1 which follows:

TABLE I

| Example Number                                 | IV    | V     | VI    | VII   | VIII  | IX    | X     | XI    | XII   |
|------------------------------------------------|-------|-------|-------|-------|-------|-------|-------|-------|-------|
| Deoxidizing solution composition: <sup>1</sup> |       |       |       |       |       |       |       |       |       |
| Potassium peroxydiphosphate (g./l.)            | 118.6 | 118.6 | 118.6 | 118.6 | 111.6 | 111.6 | 111.6 | 111.6 | 111.6 |
| Sulfuric acid (66° Bé.) (ml./l.)               | 40.0  | 40.0  | 40.0  | 40.0  | 40.0  | 40.0  | 40.0  | 40.0  | 40.0  |
| NaF (g./l.)                                    | 2.4   |       |       |       | 8.4   |       |       |       |       |
| Na <sub>2</sub> HF <sub>2</sub> (g./l.)        |       | 2.4   |       |       |       | 8.4   |       |       |       |
| NH <sub>4</sub> HF <sub>2</sub> (g./l.)        |       |       | 2.4   |       |       | 8.4   |       |       |       |
| Na <sub>2</sub> SiF <sub>6</sub> (g./l.)       |       |       |       | 2.4   |       |       | 8.4   |       |       |
| HF (70%) (ml./l.)                              |       |       |       |       |       |       | 2.0   |       |       |
| pH of deoxidizing solution                     | 2.0   | 2.2   | 2.3   | 1.8   | 2.7   | 2.6   | 2.5   | 1.9   | 2.2   |

<sup>1</sup> Ingredients shown are in addition to water.

In each instance the surfaces of the resulting aluminum articles, which were smut-free and of light appearance, provided a highly satisfactory base for further finishing operations.

#### Example XIII

A dry mixture is prepared by admixing 100 g. of finely-divided sodium bisulfate and 19 g. of finely-divided sodium bisulfate and 18 g. of finely-divided potassium peroxydiphosphate. This composition, when thoroughly mixed, can be stored for long periods of time in appropriate shipping containers without hazard and without deterioration.

An aqueous solution is prepared containing 118 g. of the above-described dry mix per liter (pH about 1.6). This solution is employed in desmutting and deoxidizing articles prepared from Type 7075 aluminum alloy in the same manner as set forth in Example I. The thus-treated articles possess a light and smut-free surface highly suitable for further operations including anodizing, dyeing, painting, etc.

#### Example XIV

An acidic aqueous composition containing, in addition to water, 120 g./l. of potassium peroxydiphosphate and 40 mls. of sulfuric acid (66° Bé.) is prepared.

Aluminum articles constructed of Type 2024 and 7075 aluminum alloys are first alkaline cleaned, rinsed and then immersed in the peroxydiphosphate solution of this example for 4 minutes at a temperature of 90° F. to give smut-free articles.

What is claimed is:

1. A composition for desmutting and deoxidizing aluminum and aluminum alloys consisting essentially of a dry admixture of from about 5 to 20 weight percent of a compound selected from the group consisting of an alkali metal peroxydiphosphate, an alkaline earth metal peroxydiphosphate, and ammonium peroxydiphosphate; from about 77 to 95 weight percent of an acid salt of sulfuric acid and from 0 to about 3.0 weight percent of water-soluble fluoride salt.

2. The composition of claim 1 wherein the said compound is potassium peroxydiphosphate.

3. The composition of claim 1 wherein the said acid salt of sulfuric acid is sodium bisulfate.

4. The composition of claim 1 wherein the said fluoride salt is sodium fluoride.

5. A composition according to claim 1 consisting essentially of about 15.3 weight percent of potassium peroxydiphosphate with the balance being sodium bisulfate.

20 6. A deoxidizing and desmutting solution for aluminum and aluminum alloys consisting essentially, in addition to water: (1) a soluble peroxydiphosphate compound selected from the group consisting of ammonium peroxydiphosphate, an alkali metal peroxydiphosphate and an alkaline earth metal peroxydiphosphate in amount of about 18 g./l. up to saturation; (2) a soluble fluoride salt in amount sufficient to provide a fluoride ion concentration in the solution of from 0 to about 6 g./l. and (3) an

25

acid material selected from the group consisting of sulfuric, phosphoric and sulfamic acid, the acid salts thereof, and mixtures of the said acids and acid salts, in amount sufficient to provide a solution pH of not more than 3.0.

50 7. The solution of claim 6 wherein the said peroxydiphosphate compound is potassium peroxydiphosphate.

8. The solution of claim 6 wherein the said acid is sulfuric acid.

9. The solution of claim 6 wherein said fluoride salt is sodium fluoride.

55 10. A solution according to claim 6 consisting essentially, in addition to water, potassium peroxydiphosphate and sulfuric acid.

11. A process for deoxidizing and desmutting aluminum 60 and aluminum alloy articles which comprises treating said articles by immersing them for a period of about 1 to about 10 minutes at a temperature of about 60° F. to about 170° F. in a solution consisting essentially, in addition to water: (1) a soluble peroxydiphosphate compound selected from the group consisting of ammonium peroxydiphosphate, an alkali metal peroxydiphosphate, and an alkaline earth metal peroxydiphosphate, in amount of about 18 g./l. up to saturation; (2) a soluble fluoride salt in amount sufficient to provide a fluoride ion concentration in the solution of from 0 to about 6 g./l. and (3)

65 an acid material selected from the group consisting of sulfuric, phosphoric and sulfamic acid, and the acid salts thereof and mixtures of the said acid and acid salts, in amount sufficient to provide a solution pH of not more than 3.0.

70

75

12. The process of claim 10 wherein the said solution  
he peroxydiphosphate compound is potassium peroxy-  
diphosphate.

13. The process of claim 10 wherein the said solution,  
he said acid material is sulfuric acid.

14. The process of claim 10 wherein the said solution,  
he said fluoride salt is sodium fluoride.

15. The process of claim 10 wherein the said solution  
onsisting essentially, in addition to water, potassium  
peroxydiphosphate and sulfuric acid.

## References Cited

## UNITED STATES PATENTS

|                                   |        |          |           |
|-----------------------------------|--------|----------|-----------|
| 3,140,203                         | 7/1964 | Grunwald | 134—3     |
| 3,373,114                         | 3/1968 | Grunwald | 252—186 X |
| MAYER WEINBLATT, Primary Examiner |        |          |           |
| U.S. Cl. X.R.                     |        |          |           |

10 134—3, 22, 41, 42; 156—14, 18, 21, 22; 252—79.1, 186